

3,262,778

**ALLOYS RESISTANT TO HIGH TEMPERATURES**  
William T. Kaarlela, Fort Worth, Tex., assignor to General Dynamics Corporation, Fort Worth, Tex., a corporation of Delaware

No Drawing. Original application Apr. 9, 1963, Ser. No. 271,577, now Patent No. 3,220,828, dated Nov. 30, 1965. Divided and this application Apr. 15, 1965, Ser. No. 448,250

3 Claims. (Cl. 75—134)

This application is a division of applicant's copending application Serial No. 271,577, filed April 9, 1963, now Patent No. 3,220,828.

This invention relates in general to refractory metal alloys capable of resisting high temperatures and more particularly, to alloys of such character as may be well suited for the brazing of refractory metals such as columbium, tantalum, molybdenum, and their alloys, and having additional utility as high temperature protective coatings and as structural alloys.

It has become increasingly important particularly in missile, spacecraft and aircraft applications, to use materials which are capable of withstanding extremely high temperatures. In addition to molybdenum and tantalum, one such material is columbium, which is a refractory metal possessing a melting point in the vicinity of 4400° F. From a design standpoint, it is an excellent material because of its high strength to weight ratio in the 2000 to 2500° F. range of service temperatures. It does not strain-harden rapidly; allowing cold working up to 99% without annealing, and it is therefore particularly suitable for the forming of parts of complex shape. Columbium is also characterized by moderate density (comparable to iron and nickel), and a high melting point, with good strength retention above the useful range of currently available alloys.

Useful though it is in high temperature areas, joinder of the metal and its alloys present problems. Thus, although it may be welded, nitrogen contamination is a deleterious obstacle since it causes an increase in the tendency for crater cracking, serious loss of ductility and an increase in the transition temperature. Welding also presents the problem of loss of strength due to recrystallization. In the handling of high strength columbium alloys, recrystallization occurs between 2200° and 2800° F., depending upon the alloy makeup. Welding involves these high temperatures and where recrystallization as a result occurs, a loss of approximately 50% in tensile strength may be anticipated.

However, it has been found that by using the alloy of this invention, excellent joinder of the metals is effected and a high temperature resistant joint is produced which is compatible with the strength characteristics of the joined materials. Vacuum environment or inert atmospheres such as argon gas are utilized to prevent oxidation of the columbium and its alloys during the brazing; only moderate efforts being necessary for purification of the argon gas preparatory to brazing.

The alloy of this invention is additionally useful as a coating for columbium and for other materials characterized by low oxidation resistance at elevated temperatures, i.e., of approximately 2000° F.

Further utility for this alloy is found in structural applications, such as castings, and in other areas of service where adequate oxidation resistance at elevated temperatures is difficult to achieve and maintain and where both structural and non-structural provisions are a requirement.

Accordingly, it is an object of this invention to provide an alloy well suited for the brazing of refractory metals such as columbium, molybdenum, tantalum, and their

alloys; which alloy is capable of providing excellent joint strength at elevated temperatures.

It is another object of this invention to provide an alloy of the character described which does not require excessively high temperatures for brazing and which possesses adequate ductility.

A further object is to provide an alloy, as described, which does not cause excessive erosion of the base alloys when applied thereto in brazing applications.

10 Yet a further object is to provide an alloy suitable as a protective coating for preventing oxidation of materials having a high susceptibility thereto at elevated temperatures.

15 Another object is the provision of an alloy adapted to casting applications which calls for materials possessing adequate oxidation resistance at elevated temperatures.

These and other objects and advantages of this invention will become apparent from the following description of the alloy and its characteristics and the claims directed thereto.

20 In general the alloy of this invention includes titanium as a matrix element in the percentage-by-weight ranges indicated. This matrix element is characterized by its compatibility with columbium, molybdenum, tantalum, and the alloys thereof. The alloying elements added to the matrix element comprise chromium, columbium and germanium, and are proportioned as hereinafter set forth. The resulting alloy has produced brazed joints having joint strength at high temperatures. This brazing has been effected without the use of extremely high temperatures. The ability of the alloy to withstand high temperatures with a minimum of deterioration has contributed to its further utilization as a coating and as a barrier for protection against oxidation of various materials inherently susceptible thereto. Usable tensile strength of this alloy at temperatures around 2000° F. further dictate its use in the area of structural material, particularly in casting applications.

25 It is to be understood that percentages used herein in both specification and claims, to describe ingredient proportions, are percentages by weight unless otherwise stated.

30 Titanium as an elemental constituent of the alloy has been found to be quite compatible with the refractory metals, forming a tough, narrow, diffusion layer at the interface with the brazing alloy. As employed herein, the general range of titanium is from about 20% to about 90% by weight of the alloy. A preferred range has been found to be from 30% to about 85%. Superior alloy compositions have been established incorporating the specific proportions of titanium tabulated below.

35 Chromium, like titanium, is quite compatible with the refractory metals forming a diffusion layer at the interface with the brazing alloy. As employed herein the general range for chromium is from about 20% to about 65% by weight of the alloy. A preferred range has been found to be 30% to about 48%. Superior alloy compositions include chromium in the quantities set forth hereinafter.

40 The addition of columbium improves the toughness and ductility of the alloy, and further finds use in adjusting the alloy melting temperature and reducing the alloy erosion characteristics, while significantly increasing the high temperature strength. The general range for columbium is from about 5% to about 35%, and the preferred range is from about 10% to about 30%.

45 Germanium serves to improve oxidation resistance and depresses the melting point. For germanium, the general range is from about 5% to about 25%, and the preferred range is from about 7% to about 16%.

50 Although the process for alloy formulation is subject to considerable variation, the alloy of the present invention

tion has, for test purposes, been formulated by mixing the elemental ingredients together in the desired proportions in powder form. The mixture is subsequently briquetted into a compact; then melted in a cold-hearth, water-cooled, copper crucible. If ductile, the alloy is then rolled to form a foil, or in the alternative, broken and crushed into a powder to be used in this form.

As formulated herein, the alloy of this invention has taken the powder form. Application is effected by mixing the powder alloy with polyvinyl alcohol in a slurry, which is then painted on the joint to be brazed. The alloy is then heated to a temperature above its melting point in a protective environment, such as in a vacuum or using an argon atmosphere or other suitable inert gases for protection against the detrimental effect of oxidation. As hereinabove stated, moderate efforts should be made to purify the argon gas, if best results are to be obtained. This has been accomplished satisfactorily, in the present instance, by passing the argon through a -100° F. Dry Ice-acetone cold trap, and a closed zirconia tube filled with titanium strips and operating at 1750° F. The protection offered by the inert argon gas is important. Should atmospheric contamination occur it will be directly reflected in reduced flow and wetting of the brazing alloy, resulting in an inferior joint.

For purposes of the tests, the results of which are reflected in the tabulations below, brazed lap shear test specimens are made up using a columbium alloy incorporating by weight 10% titanium and 10% molybdenum. These were employed as the members to be joined and lap shear tested. Time at temperature prior to testing was 1-5 minutes. Employing an A-frame type lap shear tension test apparatus, failure was made to occur within one minute by steadily increasing the mechanical stress upon the specimen by means of a floating screw. Test temperatures were effected by the induction heating of a graphite susceptor surrounding the specimen. Stress was measured by means of a calibrated load link in conjunction with a strain recorder. Specimens were confined under protective, substantially inert, argon atmosphere during heating, testing and cooling.

The alloy of this invention is set forth in the table below with an indication both as to the general range of its ingredients and as to the specific composition of the particular alloy tested:

| Element  | Ti    | Cr    | Ge   | Cb   |
|----------|-------|-------|------|------|
| General  | 20-65 | 20-65 | 5-25 | 5-35 |
| Specific | 35    | 35    | 10   | 20   |

Further, the alloy was tested for structural integrity, brazing characteristics and environmental resistance. Such values as brazing temperature, re-melt temperature,

shear strength, toughness factor and brazeability on columbium, molybdenum and tantalum were established and are set forth in tabular form below:

| 5 | Braze Temp.<br>in ° F. | Joint Remelt<br>Temp., ° F.,<br>on Cb | Shear Strength in<br>Cb Joint in p.s.i. |            | Brazeability |        |        |                |
|---|------------------------|---------------------------------------|-----------------------------------------|------------|--------------|--------|--------|----------------|
|   |                        |                                       | 72°                                     | 2,000°     | On Cb        | On Mo  |        |                |
|   |                        |                                       | 10                                      | 2,650..... | +3,600       | 29,800 | 21,200 | Excel... Good. |
|   |                        |                                       |                                         |            |              |        |        |                |

15 During these tests, a remelt temperature rise phenomenon was observed in connection with the alloy in the above tabulation of test results. That is to say the brazing temperature of the alloy was 2650° F. However, in tests after brazing of the columbium T specimens, it 20 was found that the alloy did not remelt up to a temperature of more than 3500° F.

25 Thus, a highly useful titanium-chromium based alloy having columbium and germanium for braze joining or coating of refractory metals, particularly where high temperature use is contemplated, has been devised, yet one which permits brazing to be accomplished at a temperature which is not harmful to the structure, has a minimal oxidation and erosion characteristic on the joined parts, and achieves high temperature strength.

30 I claim:

1. An alloy characterized by its ability to withstand high temperatures and consisting of from about 20% to about 65% titanium, from about 20% to about 65% chromium, from about 5% to about 35% columbium, and from about 5% to about 25% germanium.
2. An alloy characterized by its ability to withstand high temperatures and consisting of from about 30% to about 48% titanium, from about 30% to about 48% chromium, from about 10% to about 30% columbium, and from about 7% to about 16% germanium.
3. An alloy characterized by its ability to withstand high temperatures and consisting of about 35% titanium, about 35% chromium, about 20% columbium, and about 10% germanium.

45

#### References Cited by the Examiner

##### UNITED STATES PATENTS

- |           |         |          |          |
|-----------|---------|----------|----------|
| 2,169,193 | 8/1939  | Comstock | 75-134.3 |
| 3,111,406 | 11/1963 | Kaarlela | 75-175.5 |
| 3,131,059 | 4/1964  | Kaarlela | 75-176   |

50 DAVID L. RECK, Primary Examiner.

55 C. N. LOVELL, Assistant Examiner.